

1

2,969,329

## DETERGENT COMPOSITIONS

Samuel Allen Heininger, Dayton, Ohio, assignor to Monsanto Chemical Company, St. Louis, Mo., a corporation of Delaware

No Drawing. Filed Apr. 12, 1956, Ser. No. 577,669

17 Claims. (Cl. 252—153)

The present invention relates to dishwashing detergents, and particularly to specific detergent compositions characterized by reduced tarnishing action towards metals, especially copper base alloys. An object of the present invention is the reduction of the discoloration and tarnishing of metals by certain detergent components, particularly non-ionic and anionic synthetic, organic detergent compounds. It is a further object of the invention to provide compositions containing the said components in the concentrations necessary in detergent formulations, and to the improvement of such formulations by the combination therewith of a specific tarnish inhibitor.

Another object of the invention is to provide detergent compositions which may be employed in washing soiled cutlery and dishes which remain in contact with the detergent solution for prolonged periods of time. It has been found that cutlery articles, including knives, forks, spoons and other tableware made of German silver and similar copper base alloys, are normally discolored by solutions containing high concentrations of conventional, organic, non-ionic or anionic detergent compound. This is commonly observed in the washing of soiled cutlery and other household utensils consisting of copper base alloys, particularly during air drying, under which conditions residual amounts of detergent solutions may remain in contact with the cutlery for prolonged periods of time. For example, forks and spoons exhibit tarnishing at those contact points from which the residual solution is evaporated at the conclusion of the washing operation. Plated cutlery made from a base of a copper alloy also exhibits this tarnishing if the plating is scratched or thin, and such tarnishing action may be found on the entire piece of cutlery.

It has now been found that the tarnishing or discoloration effect upon copper alloys, which is characteristic of non-ionic and anionic synthetic detergent compounds may be inhibited by the combination therewith of benzazimidol in minor proportions sufficient to inhibit the said tarnishing. A preferred proportion of benzazimidol employed to reduce discoloration and tarnishing in a detergent composition is from 0.01% to 0.5% by weight based upon the synthetic organic detergent. The mechanism of the inhibitory effect is not clear, but it has been found that relatively small proportions of benzazimidol are effective in overcoming the tarnishing effect of the chemical compounds utilized in detergent compositions.

Benzazimidol was prepared by the reaction of hydrazine hydrate upon o-nitrochlorobenzene. The preparation was carried out by placing 157 g. (1 mole) of o-nitrochlorobenzene in a 500 ml. flask and adding thereto a mixture of 250 g. (2.5 mole) of hydrazine hydrate and 47 g. of water. The reaction mixture was stirred and heated until refluxing began and was then maintained at reflux conditions for five and one-half hours, during which time the pot temperature remained at 110—112° C. During this period the original reaction charge changed from an oily, two-phase system to a clear, red solution. At the conclusion of the reaction period, the reaction mixture

2

was poured into one liter of water. The red-colored, organic layer was then extracted three times with ether to give a red-colored ethereal extract and a yellow-colored aqueous phase. The aqueous solution was then acidified with 6 M HCl, giving a thick slurry. This was filtered to yield a white solid, which was washed with ice-water and filtered again. The solid product was dried in a vacuum oven at 80° C. and was ground to give an almost white powder, weighing 120 g., M.P. 152—154° C. Upon cooling the filtrate from the above final treatment, a further yield of 7.0 g. of the crystalline needles was obtained to give a total recovery of 127 g., corresponding to a yield of 93.8%. The analysis of the benzazimidol,  $C_6H_5N_3O$ , was as follows: Analysis: C, 52.38; H, 4.23; N, 31.29. The calculated values for the above formula were: C, 53.3; H, 3.72; and N, 31.1.

The synthetic organic anionic and non-ionic detergent components employed in the present invention include the sulfate and sulfonate type compounds as typical anionic detergents. Representative compounds of the non-ionic type are the ethers and esters (including sulfur-containing derivatives and analogues) of polyalkylene glycols and polyglycerols. Mixtures of the above detergent components may also be employed.

The aliphatic sulfated or sulfonated detergents which are employed in combination with benzazimidol may have from 8 to 26 carbon atoms. Such detergents include the aliphatic, acyl-containing compounds having an acyl radical of about 8 to 26 carbon atoms such as the aliphatic carboxylic ester detergents. Examples of aliphatic anionic detergents are the sulfuric acid esters of polyhydric alcohols incompletely esterified with higher fatty acids, for example, cocoanut oil mono-glyceride monosulfate, tallow diglyceride monosulfate, the long-chain pure or mixed higher, primary and secondary alkyl sulfates, such as lauryl sulfate, cetyl sulfate, and higher fatty acid alcohol sulfates derived from reduced cocoanut oil fatty acids. Other compounds which may be used in combination with benzazimidol include the hydroxy sulfonated higher fatty esters, for example, the higher fatty acid esters of 2,3-dihydroxy propane sulfonic acid, and the higher fatty esters of low molecular weight alkyl sulfonic acids, such as the oleic ester of isethionic acid. The invention also contemplates the use of higher fatty ethanolamide sulfates, the higher fatty acid amides of amino alkyl sulfonic acids, for example lauric amide of taurine, etc. The salts of the various compounds employed in the present invention are preferably the sodium, ammonium or potassium salts.

One of the preferred types of detergent components is a sodium or ammonium sulfonate of an alkyl-substituted aromatic hydrocarbon selected from the group consisting of benzene, toluene and xylene, wherein the alkyl group has from 9 to 18 carbon atoms. The alkylaryl hydrocarbon is sulfonated and is then neutralized with a sodium, potassium or ammonium alkaline compound to obtain the corresponding sodium, potassium, or ammonium salt. In the preparation of the alkylaryl sulfonate, the alkyl group is preferably of about 10 to 12 carbon atoms average length, such as may be obtained from olefins or from kerosene. The kerosene may be chlorinated and the aromatic compound alkylated therewith in known manner. Another available composition of this type is produced by alkylating the aromatic hydrocarbon with an olefin hydrocarbon averaging 9 to 18 carbon atoms in the molecule, and thereafter sulfonating and neutralizing the product. Compounds of the sulfonate type are described in U.S. Patents 2,232,117 and 2,232,118 to Kyrides. A preferred compound of this type is sodium dodecyl benzene sulfonate, also known as sodium tetrapropyl benzene sulfonate when derived from tetrapropylene and benzene.

Other compounds of the above category of anionic detergents having utility in the present invention include the sulfated esters such as the sulfated esters of succinic acid and of sulfophthalic acid. Examples of such compounds which may be employed in the present detergent compositions are the sodium salt of dioctyl sulfosuccinate, sodium hexyl-4-sulfophthalate and octadecyl sulfophthalate. The present invention may also employ sulfonates of an acid which is esterified with a monohydric alcohol. A salt of this type of compound is sodium tridecyl  $\beta$ -sulfo-10 propionate.

Another group of useful detergent compounds are the sulfated and sulfonated anionic detergents based on alkyl phenols or long chain, fatty alcohols and tall oil condensed with ethylene oxide or propylene oxide. Examples of such compounds are the sodium, ammonium or amine (e.g., triethanolamine) salts of nonyl phenol condensed with ten moles of ethylene oxide and then sulfated, while another compound is tridecanol condensed with ten moles of ethylene oxide and then sulfated.

The anionic detergents are generally employed in the form of water-soluble salts, such as the alkali metal salts described above. However, the alkaline earth metal, ammonium, amine, and alkylolamine salts are likewise of utility in the present invention. While the sodium, potassium, ammonium and alkyloamine (e.g., mono-, di- and triethanolamine) salts are ordinarily preferred, other salts such as the lithium and magnesium salts may be used if desired. For certain purposes, as in the attainment of the maximum solubility, the ammonium and alkyloamine salts are preferred.

The non-ionic compounds which are employed in the present invention include the polyoxyethylene ethers of aliphatic alcohols having straight and branched chain configurations. Long chain derivatives of polyhydroxy compounds such as the ethers of polyalkylene glycols may also be employed in the present detergent compositions. Other compounds include the polyoxyethylene ethers of alkyl aromatic hydroxy compounds, for example, the alkylated polyoxyethylene phenols.

A typical compound of this group is the ethylene oxide condensation product of a highly branched monohydric primary alcohol such as tridecanol, having the molecular configuration of an alcohol produced by the Oxo process from an olefin such as triisobutylene or tetrapropylene, with from 1 to 20 moles of ethylene oxide per mole of alcohol. A preferred range is from 5 to 10 moles of ethylene oxide. The present invention includes the use of a mixture of isomeric monohydric primary tridecyl alcohols, said alcohols being derived from the Oxo process carried out with a material of the class consisting of polybutylenes and polypropylenes.

Another detergent component of the polyoxyethylene condensate type is the product obtained by the condensation of tall oil with ethylene oxide. The condensation of tall oil with ethylene oxide may be conducted with from 1 to 20 moles of ethylene oxide per mole of the tall oil, a preferred range being from 5 to 15 moles of ethylene oxide. Another condensation product of this type which is useful in the present invention is the product resulting from the condensation of tertiary octyl or nonyl phenol with from 5 to 20 moles of ethylene oxide per mole of the said phenol.

Polyoxyethylene compounds containing sulfur are also of utility. A compound of this type which may be employed in the present invention is the condensation product of a tertiary mercaptan having from 6 to 20 carbon atoms, condensed with from 5 to 20 moles of ethylene oxide per mole of mercaptan.

The above described polyalkylene condensation products may be prepared from propylene oxide as well as with ethylene oxide. Admixtures of these two condensing agents may also be employed.

Another synthetic, organic detergent component which may be employed in the present invention is a compound

selected from the group of alkanolamides of fatty acids, preferably having from 10 to 20 carbon atoms. A preferred compound of this type is lauric diethanolamide derived from diethanolamine and crude lauric acid. Other acids and mixtures thereof may similarly be employed for this purpose. For example, an alkanolamide may be prepared from the fatty acids derived from tall oil during the purification and fractionation thereof. The alkanolamine which is employed to form the preferred alkylolamides may be mono- or diethanolamine, mono- or diisopropanolamine, or mono- or di-n-propanolamine. Preferred amines are diethanolamine and mono-ethanolamine.

Other sources of fatty acids which may be used in the preparation of the alkylolamides are the naturally occurring fatty acids, such as those derived from cocoanut oil. The said cocoanut oil fatty acids are within the present preferred group of fatty acids having from 10 to 20 carbon atoms in the acid radical.

In addition to the above-described synthetic, organic detergent components, the present compositions may include builders such as inorganic phosphate and sulfate salts. The preferred amounts of builders are from one to twenty proportions by weight referred to the synthetic, organic detergent.

The present invention contemplates the formulation of detergent compositions including specific polyphosphates, preferred compounds being selected from the group consisting of tripolyphosphates, pyrophosphates, hexameta-phosphates, tetraphosphates, and mixtures thereof. The sodium and ammonium salts are ordinarily employed, but the potassium salts may similarly be employed, particularly in the formulation of liquid detergent concentrates. Other inorganic salts such as the sodium silicates may also be utilized in the compositions of the present invention. Detergent builders and modifiers, for example, sodium sulfate, fluorescent dyes, perfume and carboxy methyl cellulose are likewise contemplated within the scope of the invention.

The following specific examples further illustrate the present invention.

#### Example 1

A composition consisting of an intimate mixture of the following ingredients was prepared, the proportions being based on the weights of the respective components. This table also sets forth the preferred range of proportions of the respective components:

|                                       | Specific Example, Percent | Range, Percent |
|---------------------------------------|---------------------------|----------------|
| 50                                    |                           |                |
| Ammonium lauryl sulfate.....          | 10.8                      | 5-25           |
| Lauryl diethanolamide.....            | 10.4                      | 5-25           |
| Ammonium dodecyl benzene sulfate..... | 16.5                      | 5-25           |
| Ammonium sulfate.....                 | 2.3                       | 0.5-25         |
| Ethanol.....                          | 13.7                      | 0-25           |
| 55 Water.....                         | 46.37                     | 84.5-90        |
| Benzazimidol.....                     | 0.02                      | 0.01-0.5       |

A similar mixture without the benzazimidol was also prepared as a control.

The above detergent formulations were utilized in water at 0.25 weight percent concentration in order to determine the effectiveness against metal discoloration or tarnishing. The tests were conducted upon small samples of German silver which had been polished with crocus cloth, washed and rinsed in acetone. The metal test samples were tested in a half-submerged position in a beaker containing the detergent solution. The tests were conducted for a period of 24 hours at a temperature of approximately 70° F. At the conclusion of this time the metal samples were examined to determine the extent of the discoloration.

It was found that the above formulation containing benzazimidol did not appreciably discolor or tarnish the German silver. Under the same test conditions the corresponding formulation without the benzazimidol did

shows severe discoloration or tarnishing. A blank corrosion test carried out with distilled water in the absence of a detergent also showed discoloration.

*Example 2*

Tarnishing tests were conducted with 0.1 wt. percent solutions, respectively, of (a) ammonium dodecyl benzene sulfonate, (b) sodium dodecyl benzene sulfonate and (c) sodium tridecyl  $\beta$ -sulfopropionate. Samples of each detergent solution were tested by the method of Example 1, using benzazimidol at 0.2%, 0.1% and 0.08% concentration (based on the detergent), as well as control tests without the benzazimidol. It was found that all the compositions containing benzazimidol inhibited the tarnishing of German silver, while the control solutions showed pronounced tarnishing.

*Example 3*

In tests conducted to determine the effective proportions of benzazimidol in order to resist tarnishing, a series of detergent mixtures were prepared. The active components were the ethylene oxide condensation product utilizing 8.5 moles of ethylene oxide with one mole of commercial tridecanol derived from the Oxo process by the oxonation of a 12 carbon atom olefin. The discoloration tests were conducted upon samples of German silver prepared as described above. The results obtained are summarized below:

| Tridecanol—E.O., Weight, Percent | Benzazimidol, Weight, Percent | Tarnish (48 Hrs.) |
|----------------------------------|-------------------------------|-------------------|
| 0.1.....                         | 0                             | Severe.           |
| 0.1.....                         | 0.2                           | None.             |
| 0.1.....                         | 0.5                           | None.             |

The above data indicate that the combination of benzazimidol, together with a synthetic, organic detergent component resists the tarnishing effect which is otherwise characteristic of the detergent employed alone.

The detergent compositions of the present invention are of particular utility in dishwashing. It is, accordingly, an embodiment of the present invention to wash cutlery in an aqueous washing solution. The preferred concentration of the present detergent composition containing benzazimidol is from 0.05% to 0.5% by weight of the detergent product in the said dishwashing solution. The essential ingredient is the combination of a synthetic, organic detergent compound of the anionic or non-ionic type, together with a minor proportion of benzazimidol sufficient to resist tarnishing of copper base alloys by the said detergent compound.

What is claimed is:

1. A detergent composition consisting essentially of a synthetic, organic detergent selected from the group consisting of the sulfated and sulfonated anionic and non-ionic detergents, and in combination therewith a small amount of benzazimidol sufficient to inhibit tarnishing of a copper base alloy.

2. A detergent composition consisting essentially of a sulfated and sulfonated anionic, synthetic, organic detergent, and in combination therewith a small amount of benzazimidol sufficient to inhibit tarnishing a copper base alloy.

3. A detergent composition consisting essentially of a non-ionic, synthetic, organic detergent, and in combination therewith a small amount of benzazimidol sufficient to inhibit tarnishing a copper base alloy.

4. A detergent composition consisting essentially of a sodium dodecyl benzene sulfonate, and in combination therewith a small amount of benzazimidol sufficient to inhibit tarnishing a copper base alloy.

5. A detergent composition consisting essentially of an ammonium dodecyl benzene sulfonate, and in com-

bination therewith a small amount of benzazimidol sufficient to inhibit tarnishing a copper base alloy.

6. A detergent composition consisting essentially of the condensation product of 1 to 20 moles of ethylene oxide with 1 mole of tridecyl alcohol, and in combination therewith a small amount of benzazimidol sufficient to inhibit tarnishing a copper base alloy.

7. A detergent composition consisting essentially of a synthetic, organic detergent selected from the group consisting of the sulfated and sulfonated anionic and non-ionic detergents, and in combination therewith 0.01% to 0.5% of benzazimidol, based upon the said detergent, to inhibit tarnishing of a copper base alloy.

8. A detergent composition consisting essentially of a sulfated and sulfonated anionic, synthetic, organic detergent, and in combination therewith 0.01% to 0.5% of benzazimidol, based upon the said detergent, to inhibit tarnishing of a copper base alloy.

9. A detergent composition consisting essentially of a non-ionic, synthetic, organic detergent, and in combination therewith 0.01% to 0.5% of benzazimidol, based upon the said detergent, to inhibit tarnishing of a copper base alloy.

10. A detergent composition consisting essentially of a sodium dodecyl benzene sulfonate, and in combination therewith 0.01% to 0.5% of benzazimidol, based upon the said sulfonate to inhibit tarnishing of a copper base alloy.

11. A detergent composition consisting essentially of an ammonium dodecyl benzene sulfonate, and in combination therewith 0.01% to 0.5% of benzazimidol, based upon the said sulfonate to inhibit tarnishing of a copper base alloy.

12. A detergent composition consisting essentially of a condensation product of 1 to 20 moles of ethylene oxide with 1 mole of tridecyl alcohol, and in combination therewith 0.01% to 0.5% of benzazimidol, based upon the said condensation product to inhibit tarnishing of a copper base alloy.

13. An aqueous detergent bath having high detergency efficiency and being resistant to the tarnishing of a copper base alloy, consisting essentially of a synthetic, organic detergent selected from the group consisting of the sulfated and sulfonated anionic and non-ionic detergents, water, and in combination therewith about 0.01% to 0.5% by weight of benzazimidol, based upon the said detergent.

14. The method of washing cutlery which comprises subjecting said cutlery to an aqueous washing solution consisting essentially of a synthetic, organic detergent selected from the group consisting of the sulfated and sulfonated anionic and non-ionic detergents, water, and in combination therewith about 0.01% to 0.5% by weight of benzazimidol, based upon the said detergent.

15. The method of washing cutlery which comprises subjecting said cutlery to an aqueous washing solution consisting essentially of between about 0.05% to 0.5% by weight of a mixture containing as an active ingredient the condensation product of 1 to 20 moles of ethylene oxide with 1 mole of tridecyl alcohol, together with 0.01% to 0.5% by weight of benzazimidol, based upon the said condensation product.

16. A detergent composition consisting of the following ingredients in parts by weight:

|                                    | Percent  |
|------------------------------------|----------|
| Ammonium lauryl sulfate            | 5-25     |
| Lauryl diethanolamide              | 5-25     |
| Ammonium dodecyl benzene sulfonate | 5-25     |
| Ammonium sulfate                   | 0.5-5    |
| Ethanol                            | 0-25     |
| Water                              | 84.5-50  |
| Benzazimidol                       | 0.01-0.5 |

17. An aqueous detergent bath consisting essentially

of an aqueous solution of the composition defined in  
claim 1.

2,618,608 Schaeffer \_\_\_\_\_ Nov. 18, 1952  
2,733,215 Ruff \_\_\_\_\_ Jan. 31, 1956

## References Cited in the file of this patent

## UNITED STATES PATENTS

2,607,740 Vitale \_\_\_\_\_ Aug. 19, 1952  
2,618,606 Schaeffer \_\_\_\_\_ Nov. 18, 1952

## OTHER REFERENCES

Heilbron: Dictionary of Organic Compounds, volume  
II, Oxford Univ. Press, N.Y. (1953), page 734.